

## UNITED STATES PATENT OFFICE

2,439,805

METHOD OF ELECTROWINNING  
MANGANESE

Herbert R. Hanley, Rolla, Mo., and James H. Jacobs, Boulder City, Nev.

No Drawing. Application August 4, 1942,  
Serial No. 453,542

2 Claims. (Cl. 204—105)

(Granted under the act of March 3, 1883, as  
amended April 30, 1928; 370 O. G. 757)

1

This invention described herein may be manufactured and used by or for the Government for governmental purposes, without the payment to us of any royalty thereon.

Our invention relates to improvements in the art of winning manganese from aqueous solutions, and more particularly to an improved anode for use in the electrodeposition of manganese, the use of which is a marked contribution to the electrolytic managnese process.

The anode problem in the electrolytic manganese process is of vital importance. In a process where metal is plated from solutions using insoluble anodes, the choice of the material to be used in the anodes is very limited. There are two main anode reactions which might occur which would be detrimental to the process.

First, the anode must be insoluble, and second, the reactions occurring at the anode must not interfere with the process. Usually, though not necessarily, the anode product during electrolysis are oxidation compounds formed by the strong oxidizing atmosphere of probably nascent oxygen.

The first consideration, namely, the insolubility of the anodes, is very well met by the use of lead anodes in sulphate solutions. However, lead does not meet the second requirement when used in the electrolytic manganese process. When manganese sulphate-ammonium sulphate solutions are electrolyzed using lead anodes, a considerable amount of the manganese in solution is rendered insoluble, perhaps as the oxides, the main one apparently being  $MnO_2$ .

The following figures are given to show how serious this precipitation of manganese is to the electrolytic manganese process.

The Bureau of Mines reported in their electrolytic manganese work that for every three pounds of manganese produced as cathode metal there was one pound of manganese precipitated at the anodes. This amount of manganese precipitated constitutes a very serious problem, not only in keeping the electrolytic cells in proper operating condition, but finally in adding considerably to the cost of making cathode electrolytic manganese.

The following figures show how this is true:

Taking 2000 pounds of cathode metal, there would be 667 pounds of manganese precipitated at the anodes as insoluble manganese compound. The precipitate assays approximately 40% Mn, so there would be 1334 pounds of dry manganese compounds suspended in the cell anolyte. It would be necessary to filter these compounds from the anolyte, and as the wet filter cake assays at

least 50% moisture, there would be roughly 2600 pounds of the wet cake. In order to wash the ammonium sulphate bearing anolyte from the wet cake at least one ton of water would be necessary.

5 This water wash would be a problem, and it is very possible that evaporation of it would be necessary in order to keep down plant solution volumes.

In order to recover the manganese in the wet 10 filter cake a reduction roast would be necessary to convert the high manganese compounds, such as  $MnO_2$ , to the acid soluble oxide  $MnO$ .

The manganese oxides on precipitating in the 15 electrolytic cells also offer a serious problem in the fouling of the diaphragm coverings. Also, periodically, the cells would have to be shut down and cleaned of the manganese oxides which build up in the cell bottoms.

The above explanation makes clear the desirability of obtaining an anode which will prevent 20 the precipitation of the manganese compounds. This kind of anode would definitely cut down on the cost of producing electrolytic manganese.

There is one other feature in the electrolytic 25 manganese process, as it now stands, which is very undesirable and which can be overcome by use of an anode which would not allow precipitation of the oxides of manganese.

As the process is now operated the anodes and 30 cathodes are separated by cloth diaphragms. The reason for this is that manganese cannot be plated commercially from highly acid solutions. In the electrolytic cell arrangement the cathodes are placed inside the diaphragms and the anodes outside the diaphragms. As 27 cathodes are usually 35 used in each electrolytic cell, and as about 12 cells are necessary to produce one ton of cathode manganese per day, this means 324 cathodes. Each of these cathodes has its own independent 40 feed line, and as the solution inside the diaphragm holds only one-half cubic foot of solution it is very evident that considerable supervision must be maintained in order to properly feed the cells.

Now, with an anode which does not precipitate 45 the manganese oxides, the cathodes could be placed outside the diaphragms and the anodes inside the diaphragms. This would cut the feed lines to the cells from 27 to one and at the same time insure a more uniform solution around the 50 cathodes. The volume of solution per cathode jumps from one-half a cubic foot to four cubic feet, or eight times as much. As the cathode metal is the product from cells which is desired, the above change would make for steadier cathode 55 plating conditions, and at the same time reduce

considerably the amount of supervision necessary for cell control.

Several procedures have been suggested for overcoming the difficulties outlined hereinabove, but none has been fully satisfactory. The anodes have been covered with acid proof cloth, but this procedure is expensive and the cloth quickly deteriorates and ruptures.

Colin G. Fink (Anodes for Electrowinning Manganese, The Electrochemical Soc., Preprint 76-5, September 14, 1939) developed an alloy of lead-tin-cobalt which will prevent manganese from becoming oxidized at the anodes. However, this alloy is very expensive and difficult to prepare, as several steps are necessary in its preparation.

The principal object of our invention is the provision of a relatively inexpensive anode which will solve the problems discussed.

The anode of our invention is easy to prepare, is of comparatively low cost, is insoluble in manganese sulphate-ammonium sulphate solutions, and minimizes precipitation of manganese anodic compound. This anode comprises a lead-silver alloy and research work over a long period has proven its adaptability to the electrolytic manganese process.

A certain amount of the manganese compounds are formed initially on the alloy anode. Pre-forming is indicated and more fully discussed in the experimental data appended.

Lead-silver alloys form a eutectic mixture at approximately 2% to 2½% silver, 97½% to 98% lead (International Critical Tables, vol. 2, p. 414; Metals Handbook, Am. Soc. for Metals, 1939 ed., Cleveland, Ohio, p. 1523). We propose usually to use silver in a concentration about the eutectic or below. Experience in other fields (the use of Pb-Ag alloy anodes is old, e. g., U. S. 1,851,219; 1,759,493 and 1,587,438) seems to indicate that higher proportions of silver may be undesirable and the cost of silver would appear to render it inadvisable to exceed about 3%, so far as silver content is concerned, a proportion which we have found experimentally to give very desirable results. We, therefore, do not limit ourselves to the use of very low percentages of silver in the practice of our invention.

The practice of our invention may be illustrated by reference to actual test data given by way of example.

Several anodes were prepared by melting together 99% of lead and 1% of silver and casting the alloy so produced into an open mold. The anodes so produced analyzed approximately 1% silver, balance lead. As cast, they were  $\frac{1}{16}$ " thick, and were trimmed to have a surface area somewhat less than the surface area of the cathodes with which they were used. Several anodes so produced were mounted in a cell, and the anodes preformed by operating the cell for 24 hours. During the first four hours manganese was precipitated at such anodes, and at the end of this period the surface was covered with a blue-black film on which a dark scale had started to form. This scale increased during the pre-forming period. At the end of the period the scale was removed (care being exercised not to rupture the blue-black film) and the anodes were then weighed.

The cells, using the anodes prepared as above, were operated using a solution containing 140 grams per liter of ammonium sulphate and 25 grams per liter of manganese as the sulphate and 0.2 to 0.5 gram per liter of sulphur dioxide in the feed. A ten gram strip was taken and the anolyte

contained 15 grams per liter of manganese and the acid concentration was about 20 grams per liter. The cells were operated with a current density at the anodes of either 28 amperes or 58 amperes per square foot.

As the cell was operated there was a very small amount of manganese dioxide formed at the anode, but after the first day's operations, the anolyte was very clear. A dark brown scale built up on the anode surface as plating continued.

Compared with other anodes employed under the same conditions, the 1% silver-lead anodes so produced permitted operation at satisfactory current efficiency, that is, consistently above 15 50%, and it appears that more than adequate current efficiencies may be maintained. The tests ran were not particularly concerned with current efficiencies, however, but rather with MnO<sub>2</sub> formation and anode losses. The latter 20 were very low, and unquestionably may be reduced further by selection of most optimum conditions.

In another series of tests, we produced a number of anodes containing 2½% silver, balance 25 lead, and treated them in the same manner as described in connection with the 1% silver anodes. These also showed desirable results from the standpoint of efficiencies and costs, particularly from the standpoint of low MnO<sub>2</sub> production and low anode losses.

Other anodes containing other low percentages of silver produce the same desirable advantages, but in our experimental work we utilized primarily 1% and 2½% silver, and ran many tests to 35 determine the relative advantageous characteristics of these two embodiments.

For the benefit of those skilled in the art, we show below the results of operations over a period of approximately two weeks on certain anodes 40 produced in accordance with the invention, these anodes having been selected at random from the group produced, and being identified in the three tables by number. In the tables, C. D. stands for current density in amperes per square foot. The other symbols are conventional.

TABLE I

## Cell data

50

| Anode No. | Percent Ag | Anode C. D. | Amp. Hours Operated | Wt. Cathode Mn. g. | Wt. Anode Scale g. |
|-----------|------------|-------------|---------------------|--------------------|--------------------|
| 3         | 1          | 28          | 4725                | 3135.7             | 133.5              |
| 4         | 1          | 28          | 4725                | 3135.7             | 169.0              |
| 14        | 2.5        | 28          | 4725                | 2936.7             | 218.5              |
| 15        | 2.5        | 28          | 4725                | 2936.7             | 196.5              |
| 5         | 1          | 58          | 3363                | 1958               | 49.0               |
| 9         | 1          | 58          | 3363                | 1958               | 46.0               |
| 12        | 2.5        | 58          | 3363                | 1981.2             | 43.0               |
| 13        | 2.5        | 58          | 3363                | 1981.2             | 45.5               |

60

TABLE II

## Analysis of anode scale

65

| Anode No. | Percent Ag | Anode C. D. | Pb.  | Mn.  | Ag    | Ca   |
|-----------|------------|-------------|------|------|-------|------|
| 3         | 1          | 28          | 24.0 | 30.7 | .36   | 1.44 |
| 4         | 1          | 28          | 29.2 | 27.0 | .24   | 2.0  |
| 14        | 2.5        | 28          | 21.7 | 30.4 | .47   | 3.12 |
| 15        | 2.5        | 28          | 27.9 | 26.2 | .57   | 1.78 |
| 5         | 1          | 58          | 2.26 | 31.7 | 0.015 | 6.24 |
| 9         | 1          | 58          | 4.12 | 33.1 | 0.023 | 5.42 |
| 12        | 2.5        | 58          | 5.62 | 28.7 | .12   | 4.62 |
| 13        | 2.5        | 58          | 4.26 | 26.6 | .113  | 7.72 |

5  
TABLE III  
*Calculations from cell data*

| Anode No. | Percent Ag | Anode C. D. | Ratio of Mn in Scale to Mn Dep. | Percent Loss in Anode Wt. | Percent Loss Ag | Percent Loss Pb | Ag Loss Ton Mn | Pb Loss Ton Mn |
|-----------|------------|-------------|---------------------------------|---------------------------|-----------------|-----------------|----------------|----------------|
| 3-----    | 1          | 28          | .0130                           | 1.56                      | 2.29            | 1.53            | 0.31           | 20.0           |
| 4-----    | 1          | 28          | .0145                           | 2.43                      | 2.00            | 2.40            | 0.26           | 30.8           |
| 14-----   | 2.5        | 28          | .0223                           | 3.01                      | 2.56            | 2.05            | 0.70           | 31.6           |
| 15-----   | 2.5        | 28          | .0174                           | 2.49                      | 2.00            | 2.44            | 0.76           | 36.5           |
| 5-----    | 1          | 58          | .0079                           | .070                      | .06             | .08             | .007           | 1.12           |
| 9-----    | 1          | 58          | .0078                           | .147                      | .085            | .14             | .011           | 1.87           |
| 12-----   | 2.5        | 58          | .0062                           | .228                      | .185            | .22             | .05            | 2.42           |
| 13-----   | 2.5        | 58          | .0061                           | .151                      | .15             | .15             | .05            | 1.94           |

From the results shown in the preceding tables it can be seen that when the cells are operated with the higher current density on the anodes, the amount of scale formed is markedly decreased, thereby lowering the silver and lead loss and the amount of manganese precipitated at the anode. The average voltage for the 1.0% and 2.5% silver anodes at 28 current density was 4.00 volts, and at 58 current density it was 4.26 volts. The increased power cost due to the higher operating voltage when using the high current density on the anodes would more than be compensated for by the lower anode cost resulting from the small loss of lead and silver.

Very little difference could be determined between the efficiency of 1% and 2.5% Ag anodes and, since the initial investment would be smaller if the 1% Ag anodes were used, it is believed that on the basis of these tests, the 1% Ag anode would be the most logical composition to use. Although scale formed during the preforming in the tests, this would not be necessary in actual practice. The preforming of the anodes was done merely to keep the cells clear of precipitated manganese compounds, but it could be dispensed with without damaging the electrolytic circuit. The calcium present in the anode scale was due to gypsum crystals being precipitated upon the anode. The origin of other constituents of the scale is obvious.

The results show definite trends and represent the maximum losses that would be encountered with silver-lead anodes. It is believed that, as the time of operation is increased after the dark-brown scale is formed, the silver and lead losses would be greatly decreased. Based solely upon the results shown, however, the anodes of the present invention are definitely superior to other anodes, such as the lead anodes of the prior art, and in some respects superior to the so-called Fink anodes. The type of solution used, current densities employed, and other details of operation are entirely illustrative, as the anodes of the present invention are adapted for use under any conditions found suitable for the efficient electrowinning of manganese.

It must not be assumed that the anodes of our invention can be produced and used only in the form of cast shapes. The anodes may be extruded, rolled, drawn, extended, in short,

formed in any usual way, and may even be produced in the form of "clad" anodes wherein only the surface is lead-silver.

We have described the anodes of our invention as being cast, but they may be fabricated in any suitable way so long as their composition is substantially uniform. While an alloy of lead and silver, the latter in relatively small proportions, is eminently suitable, other alloying constituents not deleterious to the results desired, such as tin, for example, may be added, and, of course, the silver content may be increased if desired. The base of the alloy, preferably lead, must be a current conducting material insoluble in the anolyte, with or without other constituents, but containing at least a relatively small proportion of silver to minimize the formation of insoluble manganese compounds.

What we claim as new and desire to protect by Letters Patent of the United States is:

- 20 1. In the method of electrowinning manganese wherein an electrolyte of manganese and ammonium sulphate is electrolyzed in a diaphragm cell wherein the current efficiency is greater than 50%, the improvement which is characterized by employing an anode of lead alloyed with one to three percent silver and of less surface area than the cathode; initially operating the cell at an anode current density above about 28 to about 30 58 amperes per square foot, and exceeding the cathode current density due to the difference in their areas while maintaining the current efficiency above 50%; initially depositing a protective film on the anode under said operating conditions for a period of about 24 hours and continuing said electrolysis under said operating conditions for a period of about two weeks to form a scale composed principally of oxides of manganese and lead at the anode and reduce the manganese deposited as oxide on the anode to less than 1% of the metal deposited on the cathode.
- 35 2. The method as set forth in claim 1 wherein the anode current density is maintained at about 40 45 58 amperes per square foot.

HERBERT R. HANLEY.  
JAMES H. JACOBS.

#### REFERENCES CITED

50 The following references are of record in the file of this patent:

#### UNITED STATES PATENTS

| Number    | Name         | Date          |
|-----------|--------------|---------------|
| 1,759,493 | Tainton      | May 20, 1930  |
| 2,361,143 | Lente et al. | Oct. 24, 1944 |

#### OTHER REFERENCES

- 60 Transactions of the Electrochemical Society, volume 76 (1939), pages 403, 404, 421, 424.  
Transactions of the Electrochemical Society, volume 79 (1941), pages 331-345.  
Bureau of Mines Report of Investigations 3580, Sept. 1941, pages 26, 31, 32.